

## 1

2,987,425

## ACID PICKLING PROCESS

Richard Elliott Shaw, Windsor, England, assignor to Imperial Chemical Industries Limited, London, England, a corporation of Great Britain  
 No Drawing. Filed Sept. 16, 1957, Ser. No. 683,975  
 Claims priority, application Great Britain Sept. 25, 1956  
 2 Claims. (Cl. 134—28)

This invention provides an improved process for the 10 pickling in acid baths of metallic surfaces.

The pickling of metals and alloys in acid solutions is commonly undertaken to remove surface rust, scale, oxide layers, etc., to roughen or etch the metal, or to polish chemically the metal. There is frequently an evolution of fume and spray from baths used for such treatments due to the generation of hydrogen or other gas at the metal surface, or the liberation of steam or volatile acids such as hydrochloric. There is also a considerable loss of heat due to evaporation from the surface of these treatment baths when they are operated substantially above room temperature.

The evolution of acid fumes, spray and steam results in wastage of chemicals and heat, and constitutes a hazard to the health of operators and leads to corrosion of plant and buildings unless exhausting equipment is installed.

In this invention the evolution of acid spray and fume, and steam, from a tank, bath or pit, containing a solution of acid is largely eliminated by floating on the surface of the acid solution a layer of an inert substance which is liquid at the temperature of use of the acid and is substantially immiscible therewith. The loss of heat by surface evaporation of steam is markedly reduced by such a surface layer; this is particularly useful when the bath is being kept hot but not in constant use.

The substance may be, for example, a high boiling point paraffin such as liquid paraffin, petroleum jelly, a paraffin wax, an animal or vegetable oil such as lanolin, tallow or castor oil, bitumen, a low molecular weight synthetic resin, or a low melting point natural resin.

The layer-forming substance must be inert, i.e. stable at the temperature of the bath against attack by the solution in the bath, by any hydrogen generated, or by atmospheric oxygen. It must, of course, also be less dense than the acidic solution. It is preferable that it contains very little or no material volatile at the temperature of operation of the bath and it should be of such viscosity at the operating temperature of the bath that the layer will readily reform after being broken by, for example, the entry or exit of articles to the bath, or the exit of bubbles of gas or vapour.

The preferred layer-forming substances are, at the temperature of operation of the bath, liquid hydrocarbon materials such as various grades of oils, the viscosity being dependent largely on the operating temperature of the bath. It has been found that when pickled articles are withdrawn from the pickling bath through a layer of such liquid hydrocarbon material the hydrocarbon shows little tendency to cling to the article and is readily washed off. Of the liquid hydrocarbon materials those which are chemically saturated (i.e. contain no unsaturated carbon to carbon bonds) are preferred due to their high degree of stability.

The inert surface layer is effective in substantially reducing evolution of acid fumes from the bath. The following table shows the time required to decolourise a piece of alkaline phenol phthalein paper placed above a solution of 20% HCl at 95° C. covered to various depths with layers of a hydrocarbon oil having a viscosity of 8

## 2

centipoises at 95° C. A piece of the same paper was decolourised in 5 minutes by a normal atmosphere:

|   |                         |   |     |     |     |    |    |
|---|-------------------------|---|-----|-----|-----|----|----|
| 5 | Depth of layer, mm..... | 0 | 2.0 | 4.0 | 6.0 | 10 | 20 |
|   | Time/secs.....          | 4 | 50  | 65  | 70  | 80 | 95 |

Other experiments were carried out to determine the loss of hydrochloric acid from a 50% acid bath at 95° C. covered with layers of the same low viscosity oil to various depths.

|    |                                                   |       |      |      |     |     |     |     |     |
|----|---------------------------------------------------|-------|------|------|-----|-----|-----|-----|-----|
| 15 | Depth of oil layer, mm.....                       | 0.0   | 0.01 | 0.05 | 0.1 | 0.5 | 1.0 | 2.0 | 3.0 |
|    | Loss of hydrochloric acid, gms./sq. metre/hr..... | 1,130 | 209  | 97   | 70  | 41  | 13  | 5   | 4   |

The loss from the uncovered bath at room temperature was 3.3 gms./sq. metre/hour.

It is preferable for most effective reduction of heat losses and acid spray that the layer of substance should be at least 10 mm. thick.

In practice it is found that the depth of the layer can 30 be varied between fairly wide limits, these limits being dependent on the viscosity range of the materials used, the temperature of operation of the bath and the amount of foam formed at the interface between the inert substance and the aqueous acid.

35 The viscosity of the layer substance at the operating temperature can vary widely but it should preferably not exceed 100 poises. To ensure rapid removal of the layer forming substance from the metal article and to reduce drag out of the substance to a minimum the viscosity of the substance at the temperature of operation of the bath may be as low as 0.5—2 centipoises.

Although in general operating viscosities less than 100 centipoises are preferred, care should, of course, be taken that the flash point of the layer forming substance is 45 above that of the temperature of operation. For this reason a viscosity range of from 2—10 centipoises at the operating temperature is preferred.

A surprising feature of the invention is that the tendency 50 of the surface layer to cling to articles entering the bath does not seriously affect the speed at which the acid reacts with the metal. In any case this tendency may be minimised by using a layer of a substance with a low viscosity at the temperature of operation. Removal of adherent surface layer from the articles being treated may 55 also be assisted by the addition of surface active agents to the acid solution. It is preferred that the surface tension of the acid solution be reduced in this way to less than 40 dynes/cm., but the quantity of surface active agent added 60 should be less than that required to disperse or emulsify the surface layer into the acid solution.

Further, after treating metals in acid solution it is customary to rinse them in water to remove residues of acid and acidic salts, and for this purpose a rinse of cold running water is often used. When metals are treated in an acid solution covered by a surface layer as described in 65 this invention they retain, on removal from the solution, a thin film of the inert layer. It has been found that low viscosity hydrocarbon material is easily removed by a cold 70 water rinse whereas other surface layer substances, for example, paraffin wax are best removed by a hot water rinse. Where it is desired to free the metal entirely from

the surface layer substances it is best to employ an over-flowing rinse and leave the metal immersed until the surface of the rinse is clear of surface layer substances. A simple gravity type oil separator may be used to avoid wasting the surface layer substance removed in this way.

Since the inert layers of the present invention are so effective in reducing fuming from hot acid baths it is desirable to colour them, for example by adding a red dye, in order to warn operators that the baths are, in fact, hot.

The invention is illustrated by the following examples:

#### Example I

In the pickling treatment of rusty iron in 20% hydrochloric acid solution (200 gm. HCl gas/litre) in water at 90° C., a process which normally has to be carried out at a maximum temperature of 35° C., the loss of acid from a bath without surface layer was found to be 1550 gm./sq. metre/hour.

The bath was then covered with a 6 mm. thick layer of a hydrocarbon material having a viscosity of 3.5 centipoises at 90° C. and a flash point of 155° C. On continuing the pickling treatment under this surface layer the loss of acid was less than 10 gm./sq. metre/hour.

The pickling treatment was carried out in a 5 litre glass beaker lightly lagged with asbestos string. 308 watts of electricity were required to maintain a steady temperature of 90° C. without a surface layer. With the surface layer only 89 watts of electricity were required to maintain 90° C.

#### Example II

A bath was made up to the following composition:

|                                | Percent by weight |
|--------------------------------|-------------------|
| Nitric acid (S.G. 1.42)        | 11.0              |
| Hydrofluoric acid (40% HF)     | 5.0               |
| Non-ionic surface active agent | 0.1               |
| Water                          | Remainder         |

The surface active agent was an anhydrous condensation product of a long chain fatty alcohol and ethylene oxide, slightly soluble in the inert layer described below, and reduced the surface tension of the bath to 36 dynes/cm.

This bath was covered with a layer of saturated hydrocarbon material 12 mm. thick and operated at 24° C. The hydrocarbon material was an oil having a viscosity of 5.5 centipoises at the operating temperature and had a flash point of 125° C.

Titanium panels were treated in this bath for 5 minutes followed by rinsing in water and drying. All scale had been removed without noticeable evolution of acid spray or fumes from the surface of the bath, though the passage of small quantities of gaseous nitrogen oxides through the layer was, of course, not prevented.

#### Example III

A bath was made up to the following composition:

|                               | Percent by weight |
|-------------------------------|-------------------|
| Sulphuric acid (S.G. 1.84)    | 17.0              |
| Hydrochloric acid (S.G. 1.16) | 5.0               |
| Cationic surface active agent | 0.1               |
| Oil-soluble red dye           | 0.01              |
| Water                         | Remainder         |

The surface active agent was an alkyl trimethyl ammonium salt which reduced the surface tension of the bath to 30 dynes/cm.

This bath was covered with an inert layer as in Example II and heated to 60° C. Stainless steel wire was treated in this bath for 5 minutes followed by rinsing in water and drying. All scale had been removed without noticeable evolution of spray or fumes from the surface of the bath.

#### Example IV

A bath was made up to the following composition:

|                              | Percent by weight |
|------------------------------|-------------------|
| Sulphuric acid (S.G. 1.84)   | 15.0              |
| Inhibitor                    | 0.005             |
| Anionic surface active agent | 0.1               |
| Oil soluble red dye          | 0.01              |
| Water                        | Remainder         |

10 The surface active agent was a secondary alkyl sulphate which reduced the surface tension of the bath to 33 dynes/cm. The inhibitor was based on di-ortho tolyl thio urea.

15 This bath was covered with a layer of hydrocarbon material 12 mm. thick and heated to 65° C. The hydrocarbon material had a viscosity of 5.5 centipoises at the operating temperature and a flash point of 155° C. Scaly steel panels were treated in this bath for 30 minutes followed by rinsing in water and drying. All scale had been removed without noticeable evolution of spray or fume. The trace of hydrocarbon material carried over on the panels was removed without difficulty in the water rinse.

#### Example V

25 A bath was made up to the following composition:

|                                            | Percent by weight |
|--------------------------------------------|-------------------|
| Hydrochloric acid (S.G. 1.916)             | 26.0              |
| Inhibitor                                  | 0.1               |
| 30 Surface active agent (as in Example II) | 0.1               |
| Water                                      | Remainder         |

35 This bath was covered with an inert layer as in Example II. Rusty steel panels were treated in this bath for 30 minutes followed by rinsing in water and drying. All rust had been removed without noticeable evolution of spray or fume. The trace of hydrocarbon material carried over on the panels was removed without difficulty in the water rinse.

#### Example VI

40 A bath was made up to the following composition:

|                            | Percent by weight |
|----------------------------|-------------------|
| Sulphuric acid (S.G. 1.84) | 10.0              |
| Inhibitor                  | 0.005             |
| Water                      | Remainder         |

The inhibitor was based on di-ortho tolyl thio urea.

45 A layer of castor oil (S.G. 0.962-0.966 at 15° C., viscosity 700 centipoises at 25° C.) 12 mm. thick was poured over the bath. Rusty iron bolts were treated in this bath at 70° C. for 30 minutes. The bolts were withdrawn from the bath through the oil layer and rinsed. After rinsing they still showed water break and the oil layer remaining was satisfactory at a temporary protective coating for the rust free bolts.

50 There is an advantage in having a surface active agent present in the surface layer to facilitate the removal of any adherent surface layer when subsequently rinsing in water. It is an additional advantage to employ a surface active agent which is soluble both in the acid bath and in the surface layer so that the one surface active agent fulfils both functions. The surface layer can then act as a reservoir to take up any excess of surface active agent which may throw out of solution in the bath at elevated temperatures. The extent to which the surface active agent is soluble in the bath and layer respectively at the operating temperature is important. Alkyl trimethyl ammonium salts have adequate water solubility up to 100° C. to prevent the bath being denuded by solution into the layer. Some agents may be insufficiently water soluble and be preferentially dissolved by the layer which then adheres to work being processed and may become emulsified into the treatment bath.

55 What I claim is:

75 1. A process of pickling metal which comprises pro-

viding an acid pickling solution, covering all of the surface of said solution with a non-aqueous surface layer of inert liquid which is substantially immiscible with said pickling solution and substantially non-volatile and stable at the operating temperature of said solution, including in said surface layer and said pickling solution a surface active agent which is soluble in both *said* layer and said pickling solution, thereafter passing the metal to be pickled through said surface layer and into said solution, withdrawing the thus pickled metal through said surface layer, and then rinsing said metal with water whereby the surface active agent in said surface layer facilitates the removal of any adherent surface layer.

2. A process of pickling metal which comprises providing an acid pickling solution, covering all of the surface of said solution with a non-aqueous surface layer of saturated hydrocarbon which is liquid at the temperature of said solution and substantially immiscible therewith, said liquid being stable and substantially non-volatile at the operating temperature of said solution and inert with respect to the constituents of said solution, said surface layer having a viscosity of from 2-10 centipoises and a minimum thickness of at least 10 mm., including in said surface layer and said solution a surface active agent which is soluble in both *said* layer and solution, the amount of surface active agent dissolved in the solution

being sufficient to lower the surface tension to less than 40 dynes/cm., said surface active agent having sufficient solubility in said surface layer to take up any surface active agent separated out from said pickling solution, thereafter passing the metal to be pickled through said surface layer and into said solution, withdrawing the thus pickled metal through said surface layer, and then rinsing said metal with water whereby the surface active agent in said surface layer facilitates the removal of any adherent surface layer.

## References Cited in the file of this patent

## UNITED STATES PATENTS

|    |           |                               |               |
|----|-----------|-------------------------------|---------------|
| 15 | 870,508   | Hanna et al. <i>2,521-101</i> | Nov. 5, 1907  |
|    | 1,329,467 | Miskella <i>1,341-264x</i>    | Feb. 3, 1920  |
|    | 1,817,527 | Schlotter <i>A,94-1,01</i>    | Aug. 4, 1931  |
|    | 2,115,005 | Blaut <i>"</i>                | Apr. 26, 1938 |
| 20 | 2,524,825 | Pabst <i>2,521-143</i>        | Oct. 10, 1950 |
|    | 2,583,165 | Campbell <i>" -118</i>        | Jan. 22, 1952 |
|    | 2,640,767 | Easley et al. <i>" -101x</i>  | June 2, 1953  |

## OTHER REFERENCES

25 Voznesenski et al.: Chemical Abstract, vol. 37, col. 1085, 1086 (1943).